

Dec. 15, 1942.

A. B. SNOWDON

2,304,989

PRODUCTION OF WEARING APPAREL

Filed Sept. 20, 1940

Fig. 1.



Fig. 2.



INVENTOR

A. B. Snowdon

By  
Heller & Wolverine  
ATTORNEYS

## UNITED STATES PATENT OFFICE

2,304,989

## PRODUCTION OF WEARING APPAREL

Arthur Bruce Snowdon, Hillsdale, N. J., assignor  
to Celanese Corporation of America, a corpora-  
tion of Delaware

Application September 20, 1940, Serial No. 357,569

15 Claims. (Cl. 18—56)

This invention relates to the production of wearing apparel, and relates more particularly to the production of wearing apparel by shaping textile material comprising thermoplastic derivatives of cellulose.

An object of my invention is to form wearing apparel of three-dimensional shape in an economical and expeditious manner by shaping textile material comprising filaments of thermoplastic derivatives of cellulose by the use of heat and moisture.

Another object of my invention is to provide an improved process of forming three-dimensional articles of wearing apparel employing textile material comprising filaments of thermoplastic derivatives of cellulose.

A further object of my invention is the provision of an improved process of making three-dimensional articles of wearing apparel by laminating and shaping substantially flat textile material under the action of heat and moisture.

Other objects of this invention will appear from the following detailed description.

While my invention is applicable to the production of brassières, hats, caps, suspensories and other three-dimensional articles of wearing apparel, it is of particular importance in the making of brassières and will therefore be described in connection therewith.

Commonly, brassières are made by sewing together a relatively large number of small pieces of fabric. This method, aside from being complicated and cumbersome, results in an article having seams in the shaped portion which show through in an undesired manner. The seams also form ridges which may cause discomfort to the wearer.

It has been proposed to make brassières without seams by molding, by means of a suitable forming device, relatively flat textile material such as fabric comprising filaments or fibers of thermoplastic derivatives of cellulose. Under the influence of heat and pressure the filaments of thermoplastic derivatives of cellulose become sufficiently soft or plastic to assume the shape of the forming device and upon cooling harden into such shape. Because of the thermoplasticity of the fibers comprising the fabric, the articles so formed retain their shape substantially permanently and, therefore, do not become distorted when exposed to the elements. However, when subjected to repeated and vigorous washings and roping for the purpose of wringing, particularly in heated baths, there is a tendency for the shape portion to resume its

original flat form. This may be due in part to the heavy stress placed upon only part of the filaments or yarns of the fabric, while the stretched filaments receive none of the strain. In such operations there is also a slight tendency for the yarns of the fabric to slip over one another to equalize any strain, thereby tending to flatten out the three-dimensional breast-cup when part of that breast-cup is formed by distortion of the stitch shape instead of molding action.

I have now found that brassières having breast-cups without seams and which permanently retain their shape under all conditions of use can be formed simply and expeditiously by laminating and shaping, with the aid of heat and moisture, relatively flat textile material such as fabrics comprising filaments of thermoplastic derivatives of cellulose. The brassières may be formed of layers of textile material, eliminating any necessity of sewing the brassières except for hems, tapes, decorations, etc., around the edges.

In accordance with my invention the brassière is made from an assembly of fabric comprising an outer layer of fabric, hereinafter called the brassière fabric, which may be of filaments of natural silk, artificial silk or cotton or a mixture of these, an interlining comprising a fabric of filaments of a thermoplastic derivative of cellulose or a mixture of thermoplastic derivative of cellulose and cotton filaments, and an inner facing or lining which may be of the same material as the brassière fabric or of a different material, at least the interlining of the assembly should be adhesive in character under the action of heat and pressure. Preferably, however, the brassière fabric is made wholly of filaments of thermoplastic derivative of cellulose, as this material has been found to maintain the desired shape of the brassière better, and the interlining of a mixture of filaments of a thermoplastic derivative of cellulose and cotton. The thermoplastic derivative of cellulose may be any organic derivative of cellulose such as organic esters of cellulose and cellulose ethers. Examples of organic derivatives of cellulose are cellulose acetate, cellulose propionate and cellulose butyrate, while examples of cellulose ethers are ethyl cellulose and benzyl cellulose. The filaments may be present in substantially continuous lengths or they may be in the form of short or staple lengths associated together to form "spun" yarn. The textile materials may be

any suitable fabric which may be woven, circular knitted, warp knitted or netted.

In forming the laminated fabric the brassière fabric and the interlining are first lightly bound together by pressing them on a flat surface with a steam iron. Where the interlining is to extend up to the mid-portion only of the finished breast-cup, the inner edge of the interlining is pinked or sewn to the brassière fabric to prevent ravelling. The inner facing or lining, which should not extend beyond the interlining in order to avoid wrinkles in the brassière fabric, is then superposed on the joined brassière fabric and interlining with the interlining up and the whole assembly is placed in a heated flat-bed laminating press. This light laminating operation which is preferably effected at a pressure of about 50 pounds per square inch eliminates any relative slipping of the materials during the shaping operations.

The assembly, consisting of the brassière fabric, thermoplastic interlining and lining, is then given a preliminary shaping by stretching the same over a suitable mold to a degree which is in excess of that desired in the finished article. Preferably, the preliminary stretching of the assembly is effected in the presence of a small amount of moisture such as may be applied to the assembly by means of wet towels. This excessive stretching may be effected by means of a mold which is larger than the mold used in the final laminating step or, preferably, it may be effected by placing a cap over the final mold and then forcing the material over the same by hand or by mechanical means. The excessively stretched assembly is then wetted, as by spraying with water, placed in a molding and laminating machine where it is finally molded, laminated and shrunk to the desired size. For the preliminary shaping I have found that satisfactory results are obtained when the mold is heated from 275 to 325° F. whereas in the final molding temperatures of 250 to 275° F. may be used. However, the temperatures will vary not only with the nature of the derivative of cellulose present in the textile material but also with the amount of moisture and organic compounds having a plasticizing action present.

I have found that this excessive stretching and subsequent shrinking of the breast-cup prevents loss of shape, total collapse and undesirable shrinkage of the breast-cups in use. The shrinkage of the breast-cups made in accordance with this invention is at most 1 to 2% and is not noticeable to the wearer.

For the purpose of further describing my invention reference is had to the accompanying drawing wherein.

Figure 1 is a side elevational view in cross section of a device which may be used in shaping and molding a brassière, and

Figure 2 is a detail view in cross section of a cap which may be placed over the male mold elements for the purpose of giving a preliminary shape to the article being made.

In the drawing there is shown a female mold section 3 having cavities 4 corresponding to the shape of the article desired. The female mold section 3 may be provided with suitable ducts 5 through which may be circulated steam, hot water, or other suitable heating medium which ducts may have any desired number of branch lines 6 leading to the inner surface of said cavities. Besides steam, solvent vapors or other fluids may be injected into mold cavities. In place of

ducts 5 and branch line 6 there may be provided openings in which may be placed any suitable type of heating elements such as electric conductance or resistance coils or open flame burners and the like. Any suitable means may be provided for raising and lowering the female mold member as, for instance, a shaft 7 connected with a hand or mechanically operated raising and lowering mechanism as is well understood in the art. Suitably placed below the female mold section 3 is a male mold section 8 adapted to register with the female mold section. The male mold section is provided with a duct or ducts 9 connected to the surface of the male molds 11 by a plurality of branch lines 12 for the purpose of supplying heat and/or steam, water or other fluid to the working surface thereof.

Formed in the lower surface of the female mold section may be a groove 13 adapted to receive a gripping member 14 resiliently attached to the male mold section by means of shafts 15 operated against the action of springs 16. In order to obtain an excessive stretching of the textile fabric there is provided a cap 17 adapted to fit over the surface of the male mold members 11. The cap is preferably made of a material which readily conducts heat as, for example, aluminum, copper or lead.

In operation the textile material is first stretched over the male mold member 11 having the cap 17 thereon without the use of the female mold section. After this excessive stretching or shaping the cap member or members 17 are removed and the shaped material is placed over the male members 11 and subjected to the molding action of the machine employing both the male and female sections of the molding device.

It is to be understood that the foregoing detailed description is given merely by way of illustration and that many variations may be made therein without departing from the spirit of my invention.

Having described my invention, what I desire to secure by Letters Patent is:

1. Method of forming articles of wearing apparel or similar articles, which comprises imparting a three-dimensional shape to textile material comprising filaments or fibers of a thermoplastic derivative of cellulose to an extent greater than that desired in the finished article, and then subjecting the shaped textile material to a molding operation wherein said textile material is molded and shrunk to the desired shape.

2. Method of forming articles of wearing apparel or similar articles, which comprises imparting a three-dimensional shape to textile material comprising filaments or fibers of an organic derivative of cellulose to an extent greater than that desired in the finished article, and then subjecting the shaped textile material to a molding operation wherein said textile material is molded and shrunk to the desired shape.

3. Method of forming articles of wearing apparel or similar articles, which comprises imparting a three-dimensional shape to textile material comprising filaments or fibers of cellulose acetate to an extent greater than that desired in the finished article, and then subjecting the shaped textile material to a molding operation wherein said textile material is molded and shrunk to the desired shape.

4. Method of forming articles of wearing apparel or similar articles, which comprises imparting a three-dimensional shape to textile material

comprising filaments or fibers of an organic derivative of cellulose to an extent greater than that desired in the finished article, and then subjecting the shaped textile material to a molding operation in the presence of moisture wherein said textile material is molded and shrunk to the desired shape.

5. Method of forming articles of wearing apparel or similar articles, which comprises imparting a three-dimensional shape to textile material comprising filaments or fibers of cellulose acetate to an extent greater than that desired in the finished article, and then subjecting the shaped textile material to a molding operation in the presence of moisture wherein said textile material is molded and shrunk to the desired shape.

6. Method of forming articles of wearing apparel or similar articles, which comprises imparting a three-dimensional shape to an assembly of textile fabrics at least one of which contains filaments or fibers of an organic derivative of cellulose to an extent greater than that desired in the finished article, and then subjecting the shaped assembly to a molding operation in the presence of moisture wherein said assembly is molded and shrunk to the desired shape.

7. Method of forming articles of wearing apparel or similar articles, which comprises imparting a three-dimensional shape to an assembly of textile fabrics at least one of which contains filaments or fibers of cellulose acetate to an extent greater than that desired in the finished article, and then subjecting the shaped assembly to a molding operation in the presence of moisture wherein said assembly is molded and shrunk to the desired shape.

8. Method of forming articles of wearing apparel or similar articles, which comprises forming an assembly of fabrics by laminating on a flat surface a plurality of fabrics at least one of which contains filaments or fibers of an organic derivative of cellulose, stretching the assembly into a three-dimensional shape to an extent greater than that desired in the finished article, and then subjecting the shaped assembly to a molding operation in the presence of moisture wherein said assembly is molded and shrunk to the desired shape.

9. Method of forming articles of wearing apparel or similar articles, which comprises forming an assembly of fabrics by laminating on a flat surface a plurality of fabrics at least one of which contains filaments or fibers of cellulose acetate, stretching the assembly into a three-dimensional shape to an extent greater than that desired in the finished article, and then subjecting the shaped assembly to a molding operation in the presence of moisture wherein said assembly is molded and shrunk to the desired shape.

10. Method of forming articles of wearing apparel or similar articles, which comprises forming an assembly of fabrics by lightly laminating on a flat surface a plurality of fabrics at least one of which contains filaments or fibers of an organic derivative of cellulose, stretching the assembly into a three-dimensional shape to an extent greater than that desired in the finished article, and then subjecting the shaped assembly

to a molding operation in the presence of moisture wherein said assembly is molded, shrunk to the desired size and completely laminated.

11. Method of forming articles of wearing apparel or similar articles, which comprises forming an assembly of fabrics by lightly laminating on a flat surface a plurality of fabrics at least one of which contains filaments or fibers of cellulose acetate, stretching the assembly into a three-dimensional shape to an extent greater than that desired in the finished article, and then subjecting the shaped assembly to a molding operation in the presence of moisture wherein said assembly is molded, shrunk to the desired size and completely laminated.

20 12. Method of forming articles of wearing apparel or similar articles, which comprises forming an assembly of fabrics by lightly laminating on a flat surface a plurality of fabrics at least one of which contains filaments or fibers of an organic derivative of cellulose, stretching the assembly in the presence of a small amount of moisture into a three-dimensional shape to an extent greater than that desired in the finished article, and then subjecting the shaped assembly to a molding operation in the presence of moisture wherein said assembly is molded, shrunk to the desired size and completely laminated.

25

13. Method of forming articles of wearing apparel or similar articles, which comprises forming an assembly of fabrics by lightly laminating on a flat surface a plurality of fabrics at least one of which contains filaments or fibers of cellulose acetate, stretching the assembly in the presence of a small amount of moisture into a three-dimensional shape to an extent greater than that desired in the finished article, and then subjecting the shaped assembly to a molding operation in the presence of moisture wherein said assembly is molded, shrunk to the desired size and completely laminated.

14. Method of forming articles of wearing apparel or similar articles, which comprises forming an assembly of fabrics by lightly laminating 45 on a flat surface a plurality of fabrics at least one of which contains filaments or fibers of an organic derivative of cellulose, stretching the assembly in the presence of a small amount of moisture into a three-dimensional shape to an extent greater than that desired in the finished article, and then wetting the shaped assembly with water and subjecting the shaped assembly to a molding operation wherein said assembly is molded, shrunk to the desired size and completely 50 laminated.

15. Method of forming articles of wearing apparel or similar articles, which comprises forming an assembly of fabrics by lightly laminating on a flat surface a plurality of fabrics at least one of which contains filaments or fibers of cellulose acetate, stretching the assembly in the presence of a small amount of moisture into a three-dimensional shape to an extent greater than that desired in the finished article, and then wetting the shaped assembly with water and subjecting the shaped assembly to a molding operation wherein said assembly is molded, shrunk to the desired size and completely laminated.

## ARTHUR BRUCE SNOWDON.